# EUROPEAN PATENT SPECIFICATION

(11) **EP 2 263 842 B1**
(45) Date of publication and mention of the grant of the patent: **05.08.2015**
(21) Application number: 10166462.1
(22) Date of filing: 18.06.2010
(51) Int. Cl.: B28B 1/26, B28B 13/06, B28B 7/00

(54) **Method and installation for making a ceramic product.**
Verfahren und Anlage zur Herstellung eines Keramikprodukts
Procédé et installation de fabrication d'un produit céramique

(30) Priority: 19.06.2009 IT BO20090401
(43) Date of publication of application: 22.12.2010
(73) Proprietor: Sacmi Cooperativa Meccanici Imola Societa' Cooperativa, 40026 Imola (IT)
(72) Inventor: Mazzanti, Vasco, 40026 Imola (Bologna) (IT)
(74) Representative: Lanzoni, Luciano

(56) References cited:
- EP-A1- 1 747 866
- US-A- 4 591 472
- US-A- 5 427 722

## Description

This invention relates to a method and installation for making a ceramic product, in particular ceramic sanitaryware.

As is well known in this trade, ceramic sanitaryware (such as washbasins, toilet bowls, bidets and the like) are made by pressure casting a liquid mixture, known as slip, consisting of water, clay and very small quantities of other substances, in "shell" moulds made preferably of porous resin. The mould gives the article of sanitaryware the required shape and after a certain length of time (necessary to draw out the water) the article is extracted from the mould in a defined form and further processed according to a well-known sequence of steps until it is completely finished. Sanitaryware made in this way can be broadly divided into two main categories, namely: "solid cast" products and "liquid cast" products, as they are known in the jargon of the trade.

The first category of products (solid cast), typical examples of which are lidded cisterns, are thus defined because the thickness of the product wall is formed between the surfaces of the male and female parts of the mould.

The second category of sanitaryware, that is, liquid cast sanitaryware allows maximum freedom of form for the cistern and lids (referring again to this type of product). The mould may have different dimensional ratios within it and the casting cavities may be very large.

In this case, the casting cavity is not divided between a male and a female part, as in the previous case, but the walls of the product are formed by a single surface within the mould. Products of this type are made in installations of known type comprising the above mentioned mould and designed to utilize a high-pressure casting process which, in its simplest and most basic form, comprises the following steps:
- flushing the feed circuits with fresh slip;
- filling the mould at an initial pressure;
- forming the product wall thickness with pressure profiles greater than the filling pressure;
- emptying the mould and returning, normally, to atmospheric pressure;
- consolidating the product;
- extracting the product after opening the mould parts.

Immediately after being demoulded, the product is easily subject to plastic deformation and is referred to as "greenware" in the jargon of the trade.

The casting cycle starts with the mould closed and the moulding cavity perfectly clean and empty and ends with the mould closed but with the cavity containing the product just made and whose mechanical strength must be sufficient for it to bear its own weight when it is extracted from the mould.

In order to be complete, the production cycle must, as is known, include a step of closing the mould prior to casting, and a step of demoulding the product after it has been formed.

This type of casting, known as high-pressure casting, allows the product wall "thickness" to be formed in a relatively short space of time and appreciably reduces the overall production time. One example of an installation and related high-pressure process for making solid-cast products is known from document US 4,591,472, which describes a method and an installation according to the preamble of claims 1 and 8.

In that solution, the "female" mould is provided with two separate channels at the bottom of it, one for feeding in the slip and the other for discharging the used slip after the thickness of the ceramic product has been formed. The slip can be discharged more quickly by introducing air into the mould cavity via the slip feed channel.

One of the drawbacks of the prior art method and related installations of this type is that the structure of the ceramic ware (that is, the thickness of the cast) is formed as the water in the slip fed in at high pressure is forced out of the product and drained out through the walls of the porous mould at a rate such as to diversify the moisture gradient along the thickness of the cast. This problem cannot be solved by prior art processes and installations which, in practice, simply attempt to optimize the operating pressures between the cavity on the inside and the draining parts on the outside in order to make the thickness of the product as uniform as possible while casting is in progress.

Thus, during and after the formation of the thickness, the moisture content, or gradient, rises considerably from the surface of the cast that is in contact with the mould to the opposite surface of the cast.

In other words, the final cross section of the cast (that is, when the cast has reached the desired thickness, estimated using defined process parameters based on the shape and size of the ceramic ware to be made) can be divided into a "drier" (outermost) part and an inner part where the moisture content of the cast is still high compared to that of the drier part.

The above applies to both solid cast and liquid cast ceramic ware, though it acquires more critical proportions in products of the latter type, which tend to have more complex surfaces and intricate geometries.

This steep moisture differential, or gradient, creates stress differences in the casts during the subsequent step of drying proper, which may eventually lead to cracking and other defects, making it necessary for the product to be scrapped. The casting cycle normally includes steps of pre-drying the cast by allowing it to stand for specified lengths of time, which, however, not only do not significantly reduce the moisture gradient but tend to cause the outer surface of the cast to solidify to a greater extent than the inner portion without effectively reducing the moisture differential through the cross section of the cast. This invention therefore has for an aim to overcome the above mentioned drawbacks by providing a method for making a ceramic product which is capable of reducing the overall moisture content of the product while remaining within standard process cycle times.

Another aim of the method according to the invention is to harmonize, or at least make more uniform, the moisture content in all the sections of the product just cast.

A further aim of the invention is to provide a method for making ceramic products where the uniformity of the moisture content is obtained without modifying the basic structure of the casting installations and moulds used to make the ceramic products. Accordingly, this invention achieves this aim by providing a method and an installation for making ceramic products, in particular for making ceramic sanitaryware and comprising the technical characteristics set out in claims 1 and 8.

The technical features of the invention, with reference to the above aims, are clearly described in the claims below and its advantages are more apparent from the detailed description which follows, with reference to the accompanying drawings which illustrate a preferred embodiment of the invention provided merely by way of example without restricting the scope of the inventive concept, and in which:
- Figure 1 is a schematic representation, with some parts cut away in order to better illustrate others, of an installation for making ceramic products in which the method for making the ceramic products can be applied;
- Figure 2 is a schematic top plan view, with some parts cut away to better illustrate others, of the mould used in the installation of Figure 1;
- Figure 3 illustrates a scaled-up detail from Figure 2;
- Figure 4 is a Cartesian graph representing a controlled sequence of a step in the method according to the invention.

With reference to the accompanying drawings, in particular Figures 1 and 2, the method according to the invention is used for manufacturing ceramic products, in particular but not limited to, ceramic sanitaryware (such as, for example, washbasins, washbasin pedestals, toilet bowls, bidets, shower trays, and the like) using a liquid mixture known as slip.

The method is used in installations such as that illustrated in Figures 1 and 2, which show only the parts relevant to this invention.

The installation, denoted in its entirety by the numeral 5, basically comprises:
- a porous mould 1 comprising at least two parts 2, 3 which can be coupled to each other to form at least one cavity 4 for casting the ceramic product M;
- a unit 6 for feeding/discharging the liquid mix or slip at predetermined pressures and comprising a first pipe 7 connected at one end to a tank 8 containing the slip and at the other, to at least one of the parts 2, 3 of the mould 1;
- a unit 9 for controlling the product M casting cycle, connected at least to the unit 6 for feeding/discharging the slip.

As shown by way of a non-limiting example in Figures 1 to 3, the mould 1 comprises two parts 2, 3 (male and female) made of porous resin and forming three cavities 4, each used to make a washbasin pedestal (in this situation, the moulds are liquid casting moulds).

The accompanying drawings also schematically show customary controls (such as taps and solenoid valves) of the circuitry which feeds the fresh slip and discharges the used slip.

For making these ceramic products, the method according to the invention comprises the following steps:
- filling the porous mould 1, made up of the two parts 2, 3 coupled to each other to form one or more moulding cavities 4, with liquid mixture or slip at an initial pressure;
- forming the thickness S of the product M by adding more slip at a higher pressure than the initial filling pressure so that water is separated from the mixture and absorbed by the porous walls of the mould 1, that is to say, in an outward direction DE relative to the cavity 4;
- emptying the mould 1 of the excess slip and lowering the pressure until reaching a pressure value which, usually, is atmospheric pressure.

The step of emptying the excess slip is followed by a step of applying a negative pressure, indicated by the arrows D inside the cavity 4 in order to reverse the direction DE of the pressure previously applied to separate the water from the rest of the slip. The reversed direction enables the moisture content of the ceramic product M to be reduced.

In other words, applying a high negative pressure for a short time in the cavity or cavities 4 has the effect of making the moisture content along the thickness S of the cast product M more uniform, and hence of reducing the differences between the moisture contents of the product M along its thickness S, where the limit values of moisture content are those at the surface in contact with the mould (lowest moisture content) and at the innermost portion of the cavity (highest moisture content).

The negative pressure applied in the cavity 4 reduces the moisture of the innermost zone of the thickness S, thereby causing a general reduction in the moisture content through the product M as a whole.

Obviously, the step of applying a negative pressure may be performed in different ways and according to parameters that depend also on the type of product, that is to say, on the thickness of the product. Advantageously, this step of applying suction is performed during the step of pre-drying the interior (with the mould closed), which may take several minutes.

The graph of Figure 4, where the pressure values are on the ordinate axis and time (in seconds) is on the abscissa axis, shows different options.

A first option is to apply a negative pressure in a single step in a space of time T of between 1 and 100 seconds with a negative pressure value D of between 0.05 and 1 bar.

Preferably, the step of applying the negative pressure is performed in a shorter space of time T, for example between 1 and 10 seconds, again with negative pressure values D of between 0.05 and 1 bar.

The graph shows a first possibility, illustrated by the continuous line, with a time T of one second (products with reduced thickness) at a negative pressure of one bar, or, illustrated by a dashed line, with a time T of two seconds at one bar. Another possibility is that of performing the step of applying a negative pressure D in at least two sub-steps S1 and S2 separated by a pause P.

The dot-dashed lines in the graph show by way of a non-limiting example a first sub-step S1 of applying a negative pressure D in a space of time T1 of between 1 and 50 seconds (in this particular case, 3 seconds) and a second sub-step S2 performed in a space of time T2 again of between 1 and 50 seconds (in this case, one and a half seconds, for example) separated by a short pause P.

The two sub-steps S1 and S2 of applying the negative pressure D may, again, be performed with negative pressure values D of between 0.05 and 1 bar: as shown in the graph, the negative pressure applied in both the sub-steps S1 and S2 may be one bar.

According to the invention, the installation 5 described above comprises a unit 10 for generating the negative pressure D (illustrated as a block) equipped with a second pipe 11 leading into the cavity or cavities 4.

The unit 10 applies suction which extracts gaseous fluid through the second pipe 11 from the inside of the cavity 4 when the latter is emptied of the residual slip.

In practice, the unit 10 extracts gaseous fluid in a direction D opposite the above mentioned direction DE in which the watery part is separated from the rest of the slip while the thickness of the product is being formed.

The unit 10 is connected to and controlled by the casting control unit 9 of the installation 5 to enable suction to be applied after the cavity has been emptied of the used or residual slip.

In the embodiment illustrated purely by way of an example, the pipe 11 is connected to and passes through one of the parts 2, 3 of the mould 1 (in this case, the female part 3) and leads into the cavity 4 in a different zone from that of the first pipe 7 for feeding / discharging the slip.

More specifically, the second pipe 11 is connected to and passes through the top of the female mould part 3 on the side opposite that where the first pipe 7 is positioned.

Obviously, in the embodiment illustrated, there are three second pipes 11 leading into the respective cavities 4 of the mould 1.

The control unit 9 activates the negative pressure D after the used slip is discharged and the first pipe 7 is shut off to prevent any slip from flowing back into the cavity 4.

A method and an installation as described above, fully achieve the above mentioned aims thanks to the negative pressure in the product moulding cavity which partly dries the inner portions of the product or, rather, reduces the overall moisture content, making the moisture content more uniform along the thickness of the product.

The negative pressure is applied for a very short length of time compared to the total pre-drying time and does not therefore have a negative effect on process times but does significantly reduce the stresses on the product when it is removed from the mould and thus reduces the risk of having to scrap the product.

The invention described above is susceptible of industrial application and may be modified and adapted in several ways without thereby departing from the scope of the inventive concept defined by the claims. Moreover, all the details of the invention may be substituted by technically equivalent elements.

## Claims

1. A method for making ceramic products, the method comprising at least the following steps:
- filling a porous mould (1), made up of at least two parts (2, 3) coupled to each other to form at least one moulding cavity (4), with fluid mixture or slip under pressure;
- forming the thickness (S) of the ceramic product (M) by pouring in more slip in such a way as to separate water from the mixture and drain this water out through the walls of the mould (1), that is to say in a direction (DE) outwards from the cavity (4);
- emptying the excess slip out of the mould (1) ; the method being **characterized in that**, after the step of emptying the excess slip, it comprises a step of applying a negative pressure (D) inside the cavity (4) in order to enable the moisture content of the ceramic product (M) to be reduced.

2. The method according to claim 1, **characterized in that** the step of applying a negative pressure (D) is performed according to predetermined times by a control unit (9) in order to make the moisture content along the thickness (S) of the cast product (M) more uniform.

3. The method according to claim 1, **characterized in that** the negative pressure is applied in a single step in a space of time (T) of between 1 and 100 seconds with a negative pressure value (D) of between 0.05 and 1 bar.

4. The method according to claim 1, **characterized in that** the negative pressure is applied in a single step in a space of time (T) of between 1 and 10 seconds with a negative pressure value (D) of between 0.05 and 1 bar.

5. The method according to claim 1, **characterized in that** the step of applying a negative pressure (D) is divided into at least two sub-steps (S1, S2) separated by a pause.

6. The method according to claim 5, **characterized in that** the first sub-step (S1) of applying a negative pressure is performed in a space of time (T1) of between 1 and 50 seconds and the second sub-step (S2) is performed in a space of time (T1) of between 1 and 50 seconds.

7. The method according to claim 5, **characterized in that** the first and second sub-steps (S1, S2) of applying the negative pressure are performed at negative pressure values (D) of between 0.05 and 1 bar.

8. An installation for making a ceramic product according to the claims from 1 to 7, the installation (5) comprising at least:
- a porous mould (1) comprising at least two parts (2, 3) which can be coupled to each other to form the cavity (4) for casting the ceramic product (M);
- a unit (6) for feeding/discharging the slip at predetermined pressures and comprising a first pipe (7) connected at one end to a tank (8) containing the slip and at the other, to at least one of the parts (2, 3) of the mould (1) ;
- a unit (9) for controlling the product (M) casting cycle, connected at least to the first unit (6) for feeding/discharging the slip, **a unit (10) for generating a negative pressure (D) controlled by the control unit (9), the installation being characterized in that the unit (10) for generating a negative pressure (D) is** equipped with a second pipe (11) leading into the cavity (4) made by the mould (1) in order to extract fluid from the inside of the cavity (4) **and is configured to be activated after the used slip is discharged and the first pipe (7) is shut off to prevent any slip from flowing back into the cavity (4).**

9. The installation according to claim 8, **characterized in that** the second pipe (11) is connected to and passes through one of the parts (2, 3) of the mould (1) and leads into the cavity (4) in a different zone from that of the first pipe (7) for feeding/discharging the slip.

10. The installation according to claim 8, **characterized in that** the second pipe (11) is connected to and passes through one of the parts (2, 3) of the mould (1) in a zone of the cavity (4) opposite that where the first pipe (7) is positioned.

11. The installation according to any of the foregoing claims from 8 to 10, **characterized in that** the second pipe (11) is connected to and passes through a mould part (3) at the top of the latter, opposite where the first pipe (7) is positioned.

## Patentansprüche

1. Verfahren zur Herstellung von Keramikprodukten, wobei das Verfahren mindestens folgende Schritte umfasst:
- Füllen einer porösen Form (1), bestehend aus mindestens zwei Teilen (2, 3), die miteinander gekoppelt sind, um mindestens einen Formungshohlraum (4) zu bilden, mit einer Flüssigkeitsmischung oder einer geschlämmten Tonmasse unter Druck;
- Formen der Dicke (S) des Keramikprodukts (M) durch Eingießen von mehr geschlämmter Tonmasse, sodass Wasser aus der Mischung abgeschieden und durch die Wände der Form (1) abgeführt wird, d. h. in eine Richtung (DE) außerhalb des Hohlraums (4);
- Entleeren der überschüssigen geschlämmten Tonmasse aus der Form (1); wobei das Verfahren **dadurch gekennzeichnet ist, dass** es nach dem Schritt zum Entleeren der überschüssigen geschlämmten Tonmasse einen Schritt zum Anwenden eines negativen Drucks (D) im Hohlraum (4) umfasst, um zu ermöglichen, dass der Feuchtigkeitsgehalt des Keramikprodukts (M) reduziert wird.

2. Verfahren nach Anspruch 1, **dadurch gekennzeichnet, dass** der Schritt zum Anwenden eines negativen Drucks (D) nach vorgegebenen Zeiten durch eine Steuereinheit (9) durchgeführt wird, um dafür zu sorgen, dass der Feuchtigkeitsgehalt entlang der Dicke (S) des Gussprodukts (M) gleichmäßiger ist.

3. Verfahren nach Anspruch 1, **dadurch gekennzeichnet, dass** der negative Druck in einem einzelnen Schritt in einem Zeitraum (T) von 1 bis 100 Sekunden mit einem negativen Druckwert (D) von 0,05 bis 1 bar angewandt wird.

4. Verfahren nach Anspruch 1, **dadurch gekennzeichnet, dass** der negative Druck in einem einzelnen Schritt in einem Zeitraum (T) von 1 bis 10 Sekunden mit einem negativen Druckwert (D) von 0,05 bis 1 bar angewandt wird.

5. Verfahren nach Anspruch 1, **dadurch gekennzeichnet, dass** der Schritt des Anwendens eines negativen Drucks (D) in mindestens zwei Unterschritte (S1, S2), die durch eine Pause getrennt sind, unterteilt ist.

6. Verfahren nach Anspruch 5, **dadurch gekennzeichnet, dass** der erste Unterschritt (S1) zum Anwenden eines negativen Drucks in einem Zeitraum (T1) von 1 bis 50 Sekunden durchgeführt wird und der zweite Unterschritt (S2) in einem Zeitraum von 1 bis 50 Sekunden durchgeführt wird.

7. Verfahren nach Anspruch 5, **dadurch gekennzeichnet, dass** der erste und der zweite Unterschritt (S1, S2) zum Anwenden des negativen Drucks bei negativen Druckwerten (D) von 0,05 bis 1 bar durchgeführt werden.

8. Anlage zur Herstellung eines Keramikprodukts nach Anspruch 1 bis 7, wobei die Anlage (5) mindestens umfasst:
- eine poröse Form (1), bestehend aus mindestens zwei Teilen (2, 3), die miteinander gekoppelt werden können, um einen Hohlraum (4) zum Eingießen des Keramikprodukts (M) zu bilden;
- eine Einheit (6) zum Zuführen/Abführen der geschlämmten Tonmasse bei vorgegebenen Drücke und umfassend ein erstes Rohr (7), verbunden an einem Ende mit einem Tank (8), enthaltend die geschlämmte Tonmasse, und am anderen Ende mit mindestens einem der Teile (2, 3) der Form (1) ;
- eine Einheit (9) zur Steuerung des Gusszyklus des Produkts (M), verbunden mit mindestens der ersten Einheit (6) zum Zuführen/Abführen der geschlämmten Tonmasse, eine Einheit (10) zum Erzeugen eines negativen Drucks (D), gesteuert durch die Steuereinheit (9), wobei die Anlage **dadurch gekennzeichnet ist, dass** die Einheit (10) zum Erzeugen eines negativen Drucks (D) mit einem zweiten Rohr (11) ausgestattet ist, das in den aus der Form (1) bestehenden Hohlraum (4) führt, um Flüssigkeit aus dem Innenraum des Hohlraums (4) zu entziehen, und ausgelegt, um aktiviert zu werden, nachdem die gebrauchte geschlämmte Tonmasse abgeführt wurde und das erste Rohr (7) abgesperrt wurde, um den Rückfluss von geschlämmter Tonmasse in den Hohlraum (4) zu verhindern.

9. Anlage nach Anspruch 8, **dadurch gekennzeichnet, dass** das zweite Rohr (11) mit einem der Teile (2, 3) der Form (1) verbunden ist und durch diesen in den Hohlraum (4) in eine andere Zone als das erste Rohr (7) zum Zuführen/Abführen der geschlämmten Tonmasse führt.

10. Anlage nach Anspruch 8, **dadurch gekennzeichnet, dass** das zweite Rohr (11) mit einem der Teile (2, 3) der Form (1) verbunden ist und durch diesen in eine Zone des Hohlraums (4) führt, die gegenständig zu der angeordnet ist, an der das erste Rohr (7) positioniert ist.

11. Anlage nach einem der vorhergehenden Ansprüche 8 bis 10, **dadurch gekennzeichnet, dass** das zweite Rohr (11) mit einem Formteil (3) an der Oberseite des Formteils verbunden ist und durch diesen führt, das gegenständig zu der Stelle angeordnet ist, an der das erste Rohr (7) positioniert ist.

## Revendications

1. Procédé de fabrication de produits céramiques, le procédé comprenant au moins les étapes suivantes :
- remplir un moule poreux (1), composé d'au moins deux parties (2, 3) accouplées l'une à l'autre pour former au moins une cavité de moulage (4), avec un mélange fluide ou de la barbotine sous pression ;
- former l'épaisseur (S) du produit céramique (M) en versant davantage de barbotine de manière à séparer l'eau du mélange et à évacuer cette eau à travers les parois du moule (1), c'est-à-dire dans une direction (DE) allant hors de la cavité (4) ;
- vider l'excès de barbotine du moule (1) ; le procédé étant **caractérisé en ce que**, après l'étape consistant à vider l'excès de barbotine, il comprend une étape consistant à appliquer une pression négative (D) à l'intérieur de la cavité (4) afin de permettre à la teneur en humidité du produit céramique (M) d'être réduite.

2. Procédé selon la revendication 1, **caractérisé en ce que** l'étape, consistant à appliquer une pression négative, (D) est réalisée selon des durées prédéfinies par une unité de commande (9) afin de rendre plus uniforme la teneur en humidité le long de l'épaisseur (S) de la pièce coulée (M).

3. Procédé selon la revendication 1, **caractérisé en ce que** la pression négative est appliquée en une seule étape dans un laps de temps (T) compris entre 1 et 100 secondes à une valeur de pression négative (D) comprise entre 0,05 et 1 bar.

4. Procédé selon la revendication 1, **caractérisé en ce que** la pression négative est appliquée en une seule étape dans un laps de temps (T) compris entre 1 et 10 secondes à une valeur de pression négative (D) comprise entre 0,05 et 1 bar.

5. Procédé selon la revendication 1, **caractérisé en ce que** l'étape destinée à appliquer une pression négative (D) est divisée en au moins deux sous étapes (S1, S2) séparées par une pause.

6. Procédé selon la revendication 5, **caractérisé en ce que** la première sous étape (S1) d'application d'une pression négative est réalisée dans un laps de temps (Tl) compris entre 1 et 50 secondes et la seconde sous étape (S2) est réalisée dans un laps de temps (Tl) compris entre 1 et 50 secondes.

7. Procédé selon la revendication 5, **caractérisé en ce que** les première et seconde sous étapes (S1, S2) d'application de la pression négative sont réalisées à des valeurs de pression négatives (D) comprises entre 0,05 et 1 bar.

8. Installation de fabrication d'un produit céramique selon les revendications 1 à 7, l'installation (5) comprenant au moins :
- un moule poreux (1) comprenant au moins deux parties (2, 3) pouvant être accouplées l'une à l'autre pour former la cavité (4) pour mouler le produit céramique (M) ;
- une unité (6) pour alimenter/évacuer la barbotine à des pressions prédéfinies et comprenant un premier conduit (7) relié à une extrémité d'un réservoir (8) contenant la barbotine et à l'autre, à au moins une des parties (2, 3) du moule (1) ;
- une unité (9) destinée à commander le cycle de moulage du produit (M), reliée au moins à la première unité (6) pour alimenter/évacuer la barbotine, une unité (10) servant à générer une pression négative (D) commandée par l'unité de commande (9), l'installation étant **caractérisée en ce que** l'unité (10) servant à générer une pression négative (D) est équipée d'un second conduit (11) débouchant dans la cavité (4) faite par le moule (1) afin d'extraire le fluide de l'intérieur de la cavité (4), et est configurée pour être activée après que la barbotine usagée ait été évacuée et que le premier conduit (7) ait été fermé pour empêcher que la barbotine ne revienne dans la cavité (4).

9. Installation selon la revendication 8, **caractérisée en ce que** le second conduit (11) est relié à, et traverse, l'une des parties (2, 3) du moule (1) et débouche dans la cavité (4) dans une zone différente de celle du premier conduit (7) servant à alimenter/évacuer la barbotine.

10. Installation selon la revendication 8, **caractérisée en ce que** le second conduit (11) est relié à, et traverse, l'une des parties (2, 3) du moule (1) dans une zone de la cavité (4) opposée par rapport à la position du premier conduit (7).

11. Installation selon l'une quelconque des revendications précédentes de 8 à 10, **caractérisée en ce que** le second conduit (11) est relié à, et traverse, une partie supérieure de la partie (3) du moule, opposée par rapport à la position du premier conduit (7).
